# EUROPEAN PATENT SPECIFICATION

(11) **EP 1 602 742 B1**
(45) Date of publication and mention of the grant of the patent: **15.07.2009**
(21) Application number: 05011252.3
(22) Date of filing: 24.05.2005
(51) Int. Cl.: C22C 38/46, C22C 38/44, C21D 9/30

(54) **High-strength steel for large-scaled forging, and crankshaft**
Hochfester Stahl für die Herstellung von großen Schmiedestücken, insbesondere von Kurbelwellen
Acier à haute résistance pour la fabrication de grosses pièces forgées notamment de villebrequins

(30) Priority: 01.06.2004 JP 2004163638
(43) Date of publication of application: 07.12.2005
(73) Proprietor: KABUSHIKI KAISHA KOBE SEIKO SHO, Kobe-shi, Hyogo 651-8585 (JP)
(72) Inventor: Fukaya, Shogo, Takasago-shi Hyogo 676-8670 (JP); Kagawa, Yasunori, Takasago-shi Hyogo 676-8670 (JP); Fujitsuna, Nobuyuki, Takasago-shi Hyogo 676-8670 (JP)
(74) Representative: Müller-Boré & Partner Patentanwälte

(56) References cited:
- EP-A- 0 247 415
- EP-A- 1 087 030
- GB-A- 2 302 334
- US-A- 5 496 516
- US-A- 5 888 450
- US-A1- 2002 124 716

## Description

The present invention relates to a process for producing a large sized crankshaft which is suitable for use in a diesel engine or the like used in a ship or generator.

To improve outputs from diesel engines of ships or generators, and to achieve downsizing of these engines, it is required to strengthen steels, which is to be used for components thereof. Such components are generally produced by forged steels. This kind of steel for crankshafts has the maximum tensile strength of about 950 N/mm², while steels for crankshafts having the strength of 1000 N/mm² or more are required in order to meet such a requirement.

As the steel for large-scaled forgings with the strength of 1000 N/mm² or more, 3.5NiCrMo steel or the like is known which is used in rotors (see, for example, "Tetsu to Hagane", vol. 89 (2003) No. 6) . This steel has the most excellent strength, toughness, and the like, and is used as a rotor (rotating shaft) for a generator which is put under high load.

The above type of steel, however, contains the large amount of Ni, which is very expensive, as an alloying element for strengthening and toughing the steel, and is preferably subjected to a two-stage tempering process to ensure toughness, or to a specific prehardening process to minimize the grain size, resulting in a problem of high cost.

On the other hand, Cr-Mo steels, notably 34CrNiMo6 as defined in a DIN specification, 32CrMo12 as defined in the same, 42CrMo4 as defined in an ISO specification, have been hitherto used as steels for large-scaled crankshafts, which are used for parts of an engine and a transmission mechanism in the ships or the like. These types of steels have the advantage of relatively low cost because they have less content of Ni compared to the above-mentioned 3.5NiCrMo steel. In fact, however, these steels do not meet the recent requirements in terms of strength and toughness, as compared to the above type of steel. GB 2,302,334 describes a steel suited for crankshafts.

The present invention has been accomplished in view of the above-mentioned problems, and it is an object of the invention to provide a process for producing a low-cost large-scaled crankshaft with excellent strength and toughness.

This object is solved by the process as defined in the claim.

A high-strength steel for a large-scaled forging used in the invention has the principle that the steel consists of, by mass, (the contents of the following components being expressed in mass % in the same manner) C: 0.30 to 0.50 %, Si: more than 0.15 %, but not more than 0.40 %, Mn: 0.80 to 1.20 %, Ni: 0.80 to 2.5 %, Cr: 1.0 to 3.0 %, Mo: 0.35 to 0.70 %, V: 0.10 to 0.25 %, and balance: Fe and unavoidable impurities.

In the high-strength steel for a large-scaled forging used in the invention, a grain size in a metal structure of the steel is an ASTM grain size number ranging from 2 to 6. Further, the high-strength steel for a large-scaled forging used in the invention is produced by quenching under 200 °C from austenitizing-temperature and then tempering.

By forging the above-mentioned high strength steel for a large-scaled forging, a large-scaled crankshaft with desired properties is obtained. Such a crankshaft is useful as a crankshaft for a diesel engine used in a ship or generator.

In the high-strength steel for a large-scaled forging used in the invention, the Ni content is reduced as compared to that of the 3.5NiCrMo steel which has been proposed as steel for a high-strength Ni-Cr-Mo forging, leading to reduction in cost, while predetermined contents of Si, Mn, Cr, and the like are contained therein, enhancing the strength, giving rise to a steel for forgings of high quality at low cost. Further, this steel for forgings has very excellent hardenability (quenching ability). That is, this steel has an excellent property that the microstructure can be controlled to that consisting only of bainite and martensite. Using the excellent hardenability, the steel can be effectively utilized as material for large-scaled forged products. In particular, the steel is extremely useful as material for large-scaled crankshafts, including a crankshaft for a diesel engine used in a ship or generator.
Fig.1 is a graph showing a relation between an absorbed energy at the strength of 1000 N/mm², into which the determined absorbed energy is converted, and the Ni content.
Fig.2 is a graph showing a relation between the Ni content and the grain size number. Fig. 3 is a graph showing a relation between the tempering start temperature and the tensile strength TS.
Fig. 4 is a graph showing a relation between the tempering start temperature and the impact value (absorbed energy).

Under these problems, the inventors have been dedicated themselves to studying the development of steel for a forging in which the amount of Ni contained as an alloying element is reduced as compared to, in particular, 3.5NiCrMo steel known as the high-strength steel for forgings, leading to reduction in cost, and further which has the strength and toughness equivalent to those of the known steel, while being capable of exhibiting excellent hardenability, which is important in manufacturing the large-scaled high-strength forgings.

As a result, the inventors have found that the amount of Ni serving as a strengthening element in the above-mentioned steel for Ni-Cr-Mo based steels should be reduced as much as possible, while the elements including Si, Mn, Cr, and the like, should be added in appropriate amounts, thereby providing the steel for forgings with extremely excellent hardenability and with the improved strength and toughness to compensate for the shortage of strength caused by the decreased Ni amount.

That is, Ni is a very useful element for enhancing the strength and toughness of the Cr-Mo based steel, which has been used as the steel for forgings for multipurpose applications as mentioned above, and for improving the hardenability. For this reason, the Ni is the extremely useful element to the high-class Cr-Mo based steel for forging. However, since the Ni is the expensive element, an excessive increase in the Ni content would lead to an increase in cost of the steel, whereby the consumer' s requirements regarding prices cannot be satisfied. Accordingly, the invention involves the following important aims: to reduce the Ni content as much as possible, and to be capable of ensuring the strength and quenching properties equivalent to those of the conventional steel for Ni-Cr-Mo based steels. In order to accomplish the object of reducing cost by decreasing the amount of Ni, the Ni content is desirably reduced to not more than 2.5 %.

The steel for forgings used in the invention is characterized by that the Ni content is restricted as mentioned above, and that instead the alloying elements including Si, Mn, Cr, and the like are added in appropriate amounts. The reasons for restriction of a chemical component composition defined by the invention, including the above-mentioned elements, are as follows:

### C: 0.30 to 0.50 %

C is an element contributing to enhancement of the hardenability and improvement of the strength. To ensure enough strength and hardenability, the C needs to be contained in an amount of 0. 30 % or more. The excessive C content, however, extremely decreases the toughness, while enhancing formation of an inverse V-segregation in a large-scaled ingot. Accordingly, the C content is preferably reduced to not more than 0.50 %.

### Si: more than 0.15 %, but not more than 0.40 %

The element Si acts as a strength improving element, and needs to be contained in an amount exceeding 0.15 % in order to ensure enough strength. The excessive amount of Si, however, results in formation of the significant inverse V-segregation, making it difficult to obtain clean ingots. Accordingly, the Si content should be not more than 0.40 %.

### Mn: 0.80 to 1.20 %

The element Mn is an element contributing to enhancement of the hardenability and improvement of the strength. To ensure enough strength and hardenability, the Mn needs to be contained in an amount of 0.80 % or more. The excessive Mn content, however, enhances the tempering embrittlement. Accordingly, the Mn content needs to be not more than 1.20 %.

### Cr: 1.0 to 3.0 %

The element Cr is an element which is useful for enhancement of the hardenability and improvement of the toughness. To sufficiently exhibit these effects, the Cr needs to be contained in an amount of 1.0% or more. The excessive Cr content, however, forms inhomogeneous solidification, making it difficult to manufacture the clean steel. Accordingly, the Cr content needs to be not more than 3.0 %.

### Mo: 0.35 to 0.70 %

The element Mo is an element which effectively acts to improve all of the hardenability, strength, and toughness. To sufficiently exhibit these effects, the Mo needs to be contained in an amount of 0.35 % or more. If the Mo content is less than the above-mentioned amount, the inverse V-segregation is formed, which is not desirable. In contrast, since the excessive Mo content promotes micro-segregation in the ingots, and the Mo is a heavy element, gravity segregation tends to occur. Accordingly, the Mo content needs to be not more than 0.70 %.

### V: 0.10 to 0.25 %

The element V is an element which effectively acts to improve the hardenability and strength even in a small amount. To exhibit these effects, the V needs to be contained in an amount of 0.10 % or more. However, since the element V has a low equilibrium distribution coefficient, the excessive V content tends to cause the micro-segregation (normal segregation). Accordingly, the V content needs to be not more than 0.25 %.

In the steel for forgings used in the invention, preferable basic components are as mentioned above. The balance consists essentially of Fe, but the minute amounts of unavoidable impurities (including, for example, P, O, N, Al, or the like) may be allowed to be contained in the steels.

It is well known that minimizing the grain size improves the toughness of the steel material. To minimize the grain size, it is necessary to perform an austenitizing process as a precondition. That is, the austenitizing process is carried out for fining and uniforming the grain size, preceding the quenching. In the austenitizing process of the large-scaled forging, a holding time becomes long so that austenite transformation can take place inside the steel. Thus, the larger the product, the larger the difference in grain size between inside and outside tends to be, where a special process, such as multi-stage, namely, two or more stage, austenitizing process is often carried out to minimize the grain size.

On the other hand, it is well known that inclusion of the element Ni is effective in improving the toughness of the steel. The excessive Ni content, however, tends to increase the grain size, and austenite tends to remain in quenching. If the large amount of remaining austenite exists in quenching, then it is transformed into martensite in tempering, resulting in a hard and brittle structure mixed in, thus leading to deterioration in the toughness. This needs to temper again the martensite which has already been produced in the first tempering process, in a case where the certain toughness is strictly required. This is why the two-stage tempering process is often carried out.

From this viewpoint, the inventors have fully considered aiming for development of the steel which can ensure enough toughness even in coarse grains, and which suppresses the formation of the remaining austenite in quenching, without needing the special process, such as the two-stage tempering process, for the purpose of ensuring the toughness. As a result, it has been clearly found that the high-strength steel for forgings with the above chemical composition ensures enough toughness even in the metal structure having the grain size of the ASTM grain size No.6 or less, and has only to be subjected to only one-time tempering process. Note that the steel with the ASTM grain size number less than two, the grain size is significantly increased, resulting in degradation in toughness of the forged steel. Accordingly, the ASTM grain size number is at least two.

A crankshaft for a diesel engine used in a ship or generator has a journal diameter of at least about 150 mm, which is extremely large as compared to that of the vehicle (for example, about 15 mm). Since water quenching leads to a danger of cracking and breaking down in manufacturing the large-scaled forging, quenching of the large-scaled crankshaft is generally performed by oil quenching, polymer quenching, air cooling or the like. In manufacturing the large-scaled crankshaft of interest in the invention, although cooling rate in the quenching depends on a diameter of the crankshaft, it is not more than 50 °C/min in the oil quenching. More specifically, for a crankshaft with a diameter of 500 mm grade, the cooling rate is about 20 °C/min. For a crankshaft with a larger diameter than this (for example, 1000 mm), the cooling rate is much lower.

To obtain the high-strength steel for large-scaled forgings with both excellent strength and toughness, the microstructure is controlled to consist of bainite and martensite. As a result of studying a condition in which such a structure is achieved even at the quenching cooling rate of about 20 °C/min (in the case of oil quenching) so as to apply the steel to the large-scaled crankshaft with a diameter of 150 mm or more, the inventors have found out the aforesaid chemical composition.

Note that since, for a crankshaft with a much larger diameter, the desired cooling rate (20 °C/min) in the oil quenching is not often reached, the above "polymer quenching" is recommended to be carried out in this case. This polymer quenching involves cooling the steel by use of cooling solution which is produced by dissolving organic solvent, such as glycols (for example, diethylene glycol, polyethylene glycol, or the like), into water. Such polymer quenching is capable of achieving cooling rate higher than that in the oil quenching. Therefore, the polymer quenching is a cooling system useful for prevention of cracks, which might occur in the water quenching, and for achieving the higher cooling rate, for example, the cooling rate of more than 20 °C/min for the relatively large-scaled forgings.

In the quenching, the austenitized steel is subjected to quenching to under 200 °C, and then tempering from a viewpoint of completion of the transformation. If the quenching temperature (namely, tempering start temperature) exceeds 200 °C, partially austenite remains without transformation to bainite and martensite, which causes variations in properties.

A method of manufacturing the steel for the forging according to the invention is not particularly limited. The steel has only to be adjusted to predetermined chemical compositions, and then to be cast using a high-frequency melting furnace, an electric furnace, a converter, or the like in a normal manner. Performing a vacuum process after adjustment of the compositions is also effective. In the case of the steel for the large-scaled forging, ingot casting is mainly employed.

Apart from the features defined in the claim, a method of manufacturing a crankshaft using the steel for forgings, is not particularly limited. For example, the method may comprise the following steps of: melting steel with a predetermined composition in the electric furnace; removing an impurity element, such as S, and a gas component, such as O, by vacuum refining; ingot-making; forging to a bar after heating the ingot; heating the forged bar after an intermediate inspection and forging it into a shape of a crankshaft; and finish machining.

It should be noted that a free forging method (which involves forging a crank arm and a crank pin into one block, and finishing the forged block into the crankshaft shape by gas cutting and machining), and RR and TR forging methods (which involves performing forge processing in such a manner that the center axis of an ingot is aligned with a center axis of a crankshaft) are exemplified as a forge processing method for forging the material into the crankshaft. Inparticular, the latter is more preferable because high cleanness level without segregation can be obtained in the near surface region where high stress is loaded in operation, easily obtaining the crankshaft with excellent strength and fatigue property. The thus-obtained crankshaft is very useful as a crankshaft for a diesel engine used in a ship or generator.

Now, the effects and advantages of the invention will be hereinafter described more specifically by way of Example 2. It is understood that the invention is not to be limited to the following specific Example 2, and that various appropriate modifications can be devised and carried out within the applicable scope of the invention mentioned above and below, and are intended to be included in the technical scope of the invention.

### [Example]

### Example 1 (not forming part of the invention)

Steels with chemical compositions given in the following Table 1 were melted using a high-frequency melting furnace, and then cast into ingots (40 kg) each having a diameter of 132 to 158 mm and a length of 323 mm. A feeder-head part of each of the obtained ingots was cut off, and then the ingot was heated at 1230 °C for five to ten hours. Thereafter, the ingot was pressed into one second in height using an open-die forging press, and stretched to 90 mm x 90 mm x 600 mm after changing the forging direction to the transversal direction against the center line of the ingot. The thus-obtained billet was cooled in air.

### [Table 1]

After the steel was cooled to room temperature, a quenching process was carried out which simulated respective heating and cooling rates at a point located 50 mm (which is one tenth of the diameter) below the surface of the crankshaft having the diameter of 500 mm. More specifically, the steel was heated up to 870 °C at a rate of temperature increase of 40 °C/hr using a small-scaled simulate furnace, and kept at the temperature for one hour. (austenitizing process) Then, the steel was cooled at an average cooling rate of 20 °C/min to a temperature ranging from 500 to 870 °C to perform a quenching process. A tempering process was carried out at a temperature ranging from 580 to 630 °C for 13 hours, and cooling was performed by furnace cooling. Thereafter, mechanical properties of each of the thus-obtained steels were evaluated in the following manner. The grain size of the steel was measured based on the ASTM (grain size number).

### [Measurement Method of Mechanical Properties]

(A) Tensile tests were performed for each of the steels based on JIS Z2241, wherein the shape of a test piece, which is the JIS Z2201 No.14 specimen, is Φ6 × G.30. The mechanical properties [yield stress (YS), tensile stress (TS), elongation (EL), reduction of area (RA)] of the steel were measured.
(B) A Charpy impact test was performed for the type of steel with a tensile strength TS of not less than 1000 N/mm². The Charpy impact test was carried out based on JIS Z2242 to measure its absorbed energy vE, wherein the shape of a test piece employed is 2 mm V-notch based on JIS Z2202. In order to evaluate toughness at the same strength, the absorbed energy vEat (1000 N/mm²) at the strength of 1000 N/mm² was calculated by the following calculation method to evaluate the toughness.

The absorbed energies at tempering temperatures which brought about the strength of around 1000 N/mm² are designated as Eu and Ed, and the respective tensile strengths as Su and Sd.
Eu: Absorbed energy at an tempering temperature (Td) at which the strength of not less than 1000 N/mm² was obtained
Su: Tensile strength on the above condition
Ed: Absorbed energy at an tempering temperature (Td) at which the strength of not more than 1000 N/mm² was obtained
Sd: Tensile strength on the above condition $vEat \left(1000 N/{mm}^{2}\right) = Eu + \left(Ed-Eu\right) / \left(Su-Sd\right) \times \left(Su-1000\right)$

These results were given in the following Table 2, together with the quenching and tempering temperatures. From the results, the following can be shown. First, it has shown that in samples of tests No.1 to 3, 13, and 14, any of chemical components thereof deviates from a range specified by the invention, and that the tensile strength TS of each of these samples does not reach 1000 N/mm² (unachievable strength).

In contrast, it has shown that samples of tests No. 4 to 12, which meet the range specified by the invention, have the tensile strength of not less than 1000 N/mm². Moreover, it has found that a Charpy absorbed energy of each of these samples vE tends to depend on the Ni content.

Note that, after the austenitizing, quenching and tempering processes, a cross section of each sample was etched by natal, and then two or more views thereof were photographed by an optical microscope with a magnification of 100 times. From the photographs, area fractions of respective areas classified into ferrite and pearlite were determined to examine the metal structure of each sample. It has found that the area fractions of ferrite and pearlite in each sample are substantially zero, and the structure thereof consists essentially of bainite and martensite.

### [Table 2]

Based on such results, a relation between an absorbed energy at the strength of 1000 N/mm², into which the determined absorbed energy is converted, and the Ni content is shown in Fig.1. Further, a relation between the Ni content and the grain size number is shown in Fig.2. Fig.1 shows clearly that the steel with the Ni content of not less than 0.80 % and not more than 2.5 % has good impact property. It is generally known that increase in the Ni content improves the toughness of the steel. That is, it has shown that the effect of Ni is not exhibited markedly until the Ni content reaches 0.80 % or more. In contrast, it has shown that when the Ni content is more than 2.5 %, the toughness is lowered. This indicates, as shown in Fig.2, that the grain size increases with increase in the Ni content, and that such increase in the grain size lowers the toughness. Further, as can be seen from Figs. 1 and 2, the steel with the grain size number of two or more can ensure the good toughness. In a steel for forging in general, toughness improves monotonously as Ni content increases. However, in a combination of a composition and conditions of heat treatment, a suitable range of Ni content exists so as to maintain high toughness, as shown in this example. And the upper limit of the range of Ni content 2.5% equals by chance the aforementioned upper limit of Ni content to be considered in terms of cost.

### Example 2

Generally, in manufacturing a large-scaled forging, the steel is cooled not to room temperature, but to a temperature ranging from 200 to 300 °C, and then a tempering process is successively carried out, from a viewpoint of preventing cracking, which might be caused by deforming and thermal stresses in the quenching and tempering processes.

From this viewpoint, in the samples of the tests No. 1 and 9 as shown in Table 2 (the steels of the types A and I as shown in Table 1), influences of the tempering start temperature (quenching end temperature) on the mechanical properties [tensile strength (TS), 0.2 % proof strength (0.2PS), elongation (EL), reduction of area (RA), absorbed energy (vE)] were examined (other conditions being the same as those of the inventive examples). The results are shown in the following Table 3. Further, based on the results, a relation between the tempering start temperature and the tensile strength TS is shown in Fig. 3, and a relation between the tempering start temperature and the impact value (absorbed energy) is shown in Fig.4.

### [Table 3]

From these results, the following can be shown. In the sample of the test No.1, the tempering start temperature does not have so much influence on the mechanical properties, while in the sample of the test No.9, the tempering start temperature has significant influence on the properties. Such results have shown that setting the tempering start temperature (quenching end temperature) to not more than 200 °C can ensure the stabilized strength without degradation in toughness.

A cause of the influence of the tempering start temperature on the tensile strength in the chemical compositions specified by the invention is not clearly known, but it is considered that the chemical compositions limited within a range specified by the invention form a partial martensitic structure, and not a complete bainitic structure, and that the tempering start temperature has the influence on formation of such a transformed structure.

**Table 1**

| Type of steel | Chemical composition (mass %) | | | | | | | | | | |
|---|---|---|---|---|---|---|---|---|---|---|---|
| | C | Si | Mn | P | S | Cu | Ni | Cr | Mo | V | Al |
| A | 0.35 | D.24 | 0.62 | 0.004 | 0.003 | 0.03 | 1.51 | 1.49 | 022 | 0.081 | 0.003 |
| B | 0.28 | 0.23 | 1.05 | 0.005 | 0.003 | 0.03 | 1.52 | 2.03 | 0.52 | 0.21 | 0.004 |
| C | 0.38 | 0.26 | 0.77 | 0.003 | 0.003 | 0.03 | 1.54 | 2.03 | 0.53 | 0.19 | 0.006 |
| D | 0.36 | 0.22 | 0.99 | 0.005 | 0.003 | 0.03 | 0.22 | 2.92 | 0.47 | 0.1 | 0.005 |
| E | 0.36 | 0.24 | 0.94 | 0.005 | 0.003 | 0.03 | 3.05 | 0.21 | 0.49 | 0.11 | 0.026 |
| F | 0.36 | 0.23 | 0.98 | 0.005 | 0.003 | 0.03 | 1.63 | 1.58 | 0.48 | 0.11 | 0.022 |
| G | 0.39 | 0.2 | 0.94 | 0.008 | 0.003 | 0.04 | 0.52 | 2.9 | 0.48 | 0.15 | 0.018 |
| H | 0.38 | 0.21 | 1.02 | 0.008 | 0.003 | 0.05 | 0.62 | 2.8 | 0.47 | 0.16 | 0.030 |
| I | 0.34 | 0.22 | 0.98 | 0.007 | 0.003 | 0.04 | 1.58 | 1.59 | 0.49 | 0.16 | 0.020 |
| J | 0.36 | 0.25 | 1.03 | 0.006 | 0.003 | 0.05 | 2.01 | 1.55 | 0.48 | 0.17 | 0.022 |
| K | 0.37 | 0.23 | 0.99 | 0.007 | 0.003 | 0.04 | 2.41 | 1.62 | 0.51 | 0.17 | 0.023 |
| L | 0.34 | 0.22 | 0.97 | 0.007 | 0.003 | 0.04 | 2.98 | 1.6 | 0.49 | 0.11 | 0.023 |
| M | 0.39 | 0.2 | 0.94 | 0.008 | 0.003 | 0.04 | 0.52 | 2.9 | 0.27 | 0.15 | 0.018 |
| N | 0.39 | 0.2 | 0.94 | 0.008 | 0.003 | 0.04 | 0.52 | 2.9 | 0.48 | 0.88 | 0.018 |

**Table 2**

| Test No. | Type of steel | Quenching temperature | Tempering temperature | Grain size No. | YS (N/mm²) | TS (N/mm²) | EL (%) | RA (%) | vE Ave. | vE at (1000N/mm²) | Remarks |
|---|---|---|---|---|---|---|---|---|---|---|---|
| 1* | A | 870 | 590 | 5 | 685 | 988 | 17.8 | 65.1 | Unachievable strength | | Conventional steel 34CrNiMo6 |
| | | | 610 | 5 | 804 | 948 | 18.6 | 65.7 | | | |
| | | | 630 | 5 | 718 | 873 | 19.9 | 69.4 | | | |
| 2* | B | 870 | 590 | 3.3 | 829 | 982 | 17.1 | 63.6 | Unachievable strength | | Influence of C |
| | | | 610 | 3.3 | 769 | 917 | 20 | 70.2 | | | |
| | | | 630 | 3.3 | 708 | 860 | 20.5 | 71.1 | | | |
| 3* | C | 870 | 590 | 3.9 | 817 | 992 | 17.7 | 65.9 | Unachievable strength | | Influence of Mn |
| | | | 610 | 3.9 | 720 | 886 | 20.1 | 706 | | | |
| | | | 630 | 3.9 | 683 | 853 | 19.9 | 70.8 | | | |
| 4* | D | 870 | 580 | 6.2 | 959 | 1122 | 16.9 | 61.8 | 22.5 | 40.5 | Influences of Ni and Cr |
| | | | 600 | 6.2 | 840 | 987 | 16.6 | 65.9 | 42.4 | | |
| | | | 620 | 6.2 | 776 | 923 | 19.5 | 70.3 | 82.1 | | |
| 5* | E | 870 | 580 | 1.15 | 986 | 1122 | 17.6 | 58.6 | 21.7 | 39.0 | Ni,Cr |
| | | | 600 | 1.15 | 939 | 1067 | 17.3 | 58.7 | 23.1 | | |
| | | | 620 | 1.15 | 898 | 1016 | 17.9 | 61.4 | 35.2 | | |
| 6 | F | 870 | 580 | 2.6 | 1048 | 1190 | 16.3 | 59.3 | 20.4 | 87.3 | - |
| | | | 600 | 2.6 | 915 | 1060 | 16.9 | 61.1 | 57.6 | | |
| | | | 620 | 2.6 | 848 | 998 | 19.3 | 65.6 | 86.3 | | |
| 7* | G | 870 | 580 | 5.15 | 976 | 1133 | 14.8 | 60.7 | 31.5 | 66.7 | - |
| | | | 600 | 5.15 | 874 | 1033 | 17.1 | 63.4 | 62.3 | | |
| | | | 620 | 5.15 | 741 | 897 | 21.1 | 69.5 | 83.3 | | |
| 8 | H | 870 | 580 | 4.05 | 994 | 1138 | 15.4 | 59.5 | 36.7 | 86.4 | - |
| | | | 600 | 4.05 | 877 | 1041 | 17.7 | 64.5 | 78.7 | | |
| | | | 620 | 4.05 | 740 | 901 | 19.3 | 68.9 | 105 | | |
| 9 | I | 870 | 580 | 4.1 | 1083 | 1214 | 16.9 | 80.4 | 25.7 | 103.1 | - |
| | | | 600 | 4.1 | 988 | 1111 | 17 | 61.7 | 79.7 | | |
| | | | 620 | 4.1 | 860 | 986 | 19.9 | 66.1 | 106 | | |
| 10 | J | 870 | 580 | 2.8 | 984 | 1103 | 15.4 | 59.5 | 33.4 | 86.8 | - |
| | | | 600 | 2.8 | 867 | 1061 | 17.7 | 64.5 | 70.7 | | |
| | | | 620 | 2.8 | 733 | 931 | 19.3 | 68.9 | 105 | | |
| 11 | K | 870 | 580 | 2.4 | 989 | 1152 | 15.4 | 59.5 | 28.7 | 76.2 | - |
| | | | 600 | 2.4 | 876 | 1053 | 17.7 | 64.5 | 64.7 | | |
| | | | 620 | 2.4 | 743 | 923 | 19.3 | 68.9 | 93 | | |
| 12* | L | 870 | 580 | 1.5 | 1106 | 1218 | 15.4 | 50.6 | 19 | 45.0 | Influence of Ni |
| | | | 600 | 1.5 | 1001 | 1125 | 16.5 | 57.7 | 27.3 | | |
| | | | 620 | 1.5 | 861 | 998 | 19.2 | 62.7 | 45.3 | | |
| 13* | M | 870 | 580 | 7.85 | 976 | 993 | 14.8 | 60.7 | Unachievable strength | | Influence of Mo |
| | | | 600 | 7.85 | 874 | 936 | 17.1 | 63.4 | | | |
| | | | 620 | 7.85 | 741 | 897 | 21.1 | 69.5 | | | |
| 14* | N | 870 | 580 | 7.85 | 976 | 975 | 14.8 | 60.7 | Unachievable strenght | | Influence of V |
| | | | 600 | 7.85 | 874 | 923 | 17.1 | 63.4 | | | |
| | | | 620 | 7.85 | 741 | 885 | 21.1 | 69.5 | | | |

| | | | | | | | | | | | |
|---|---|---|---|---|---|---|---|---|---|---|---|
| * not forming part of the invention | | | | | | | | | | | |

**Table 3**

| No | Cooling rate (°C/min) | Tempering start temperature (°C) | TS (N/mm²) | | | 0.2%PS (N/mm²) | | | EL (%) | | | RA (%) | | | vE (J) | | | | | |
|---|---|---|---|---|---|---|---|---|---|---|---|---|---|---|---|---|---|---|---|---|
| | | | 1 | 2 | ave. | 1 | 2 | ave. | 1 | 2 | ave. | 1 | 2 | ave. | 1 | 2 | 3 | 4 | 5 | ave. |
| 1 34CrNi Mo6) | 21.4 | 100 | 991 | 992 | 992 | 853 | 856 | 855 | 17.9 | 18.4 | 18.2 | 65.9 | 66.2 | 66.1 | 41 | 38 | 34 | 48 | 58 | 44 |
| | | 200 | 995 | 995 | 995 | 864 | 864 | 864 | 17.9 | 17.7 | 17.8 | 66.4 | 66.5 | 66.5 | 51 | 41 | 31 | 43 | 51 | 43 |
| | | 250 | 988 | 988 | 988 | 849 | 852 | 851 | 18.3 | 18.1 | 18.2 | 65.4 | 66.0 | 65.7 | 38 | 46 | 43 | 48 | 48 | 45 |
| 9 | 21.4 | 23 | 1111 | | 1111 | 988 | | 988 | 17.0 | | 17.0 | 61.7 | | 61.7 | 88 | 85 | 66 | - | - | 60 |
| | | 100 | 1082 | 1094 | 1088 | 960 | 968 | 964 | 16.8 | 14.9 | 15.9 | 55.6 | 49.6 | 52.6 | 80 | 69 | 77 | - | - | 75 |
| | | 150 | 1072 | 1067 | 1070 | 950 | 944 | 947 | 17.4 | 16.1 | 16.8 | 58.8 | 58.6 | 58.7 | 85 | 91 | 56 | - | - | 77 |
| | | 200 | 1061 | 1053 | 1057 | 937 | 935 | 936 | 17.0 | 16.8 | 16.9 | 61.0 | 58.4 | 59.7 | 77 | 78 | 77 | - | - | 77 |
| | | 250 | 1060 | 1050 | 1055 | 937 | 935 | 936 | 17.6 | 17.7 | 17.7 | 61.6 | 61.8 | 61.7 | 82 | 85 | 84 | - | - | 84 |

## Claims

1. A process for producing a crankshaft having a journal diameter of at least 150 mm by forging a high strength steel, wherein said steel is produced by subjecting the austenitized steel to quenching to under 200°C, and then tempering it, wherein the steel consists of, by mass, (the contents of the following components being expressed in mass % in the same manner)
C: 0.30 to 0.50 %,
Si: more than 0.15 %, but not more than 0.40 %,
Mn: 0.80 to 1.20 %,
Ni: 0.80 to 2.5 %,
Cr: 1.0 to 3.0 %,
Mo: 0.35 to 0.70 %,
V: 0.10 to 0.25 %, and
balance: Fe and unavoidable impurities, wherein a grain size of a metal structure of the steel is an ASTM grain size number ranging from 2 to 6, and wherein the microstructure is controlled to consist only of bainite and martensite.

## Patentansprüche

1. Verfahren zur Herstellung einer Kurbelwelle mit einem Laufzapfendurchmesser von mindestens 150 mm durch Schmieden eines hochfesten Stahles, wobei der Stahl durch Unterwerfen des austenitischen Stahls einem Quenchen auf unter 200°C und anschließendem Tempern hergestellt wird, wobei der Stahl, bezogen auf die Masse, besteht aus (die Gehalte der folgenden Komponenten sind in der gleichen Weise in Masse-% ausgedrückt):
| | |
|---|---|
| C: | 0,30 bis 0,50%, |
| Si: | mehr als 0,15%, aber nicht mehr als 0,40%, |
| Mn: | 0,80 bis 1,20%, |
| Ni: | 0,80 bis 2,5%, |
| Cr: | 1,0 bis 3,0%, |
| Mo: | 0,35 bis 0,70%, |
| V: | 0,10 bis 0,25%, und |
der Rest: Fe und unvermeidbare Verunreinigungen, wobei eine Korngröße einer Metallstruktur des Stahls eine ASTM-Korngrößenzahl in dem Bereich von 2 bis 6 ist, und wobei die Mikrostruktur kontrolliert wird, nur aus Bainit und Martensit zu bestehen.

## Revendications

1. Procédé de production d'un vilebrequin ayant un diamètre de tourillon d'au moins 150 mm, par forgeage d'acier à haute résistance, dans lequel ledit acier est produit en soumettant l'acier austénitisé à un refroidissement à moins de 200 °C, puis en le trempant, dans lequel ledit acier est constitué par, en masse (les teneurs des composants suivants étant exprimées en % en masse de la même manière) :
C : de 0,30 à 0,50 %,
Si : plus de 0,15 % mais pas plus de de 0,40 %,
Min : de 0,80 à 1,20 %,
Ni : de 0,80 à 2,5 %,
Car : de 1,0 à 3,0 %,
Mo : de 0,35 à 0,70 %
V : de 0,10 à 0,25 % et
Solde : Fe et impuretés inévitables, dans lequel une grosseur de grain d'une structure métallique de l'acier va de 2 à 6 selon ASTM, et dans lequel la microstructure est contrôlée pour être constituée uniquement de bainite et de martensite.
